

# UNITED STATES PATENT OFFICE.

HELLMUTH REINHARDT ROSENBAUM, OF BROOKLYN, NEW YORK.

## METHOD OF AND MEANS FOR EXTENDING THE USABLE CONDITION OF METALLIC DIES AND TOOLS.

1,340,913.

Specification of Letters Patent. Patented May 25, 1920.

No Drawing.

Application filed September 2, 1918. Serial No. 321,170.

To all whom it may concern:

Be it known that I, HELLMUTH REINHARDT ROSENBAUM, a citizen of Germany, and resident of the borough of Brooklyn, county of Kings, and State of New York, have invented a new and useful Method of and Means for Extending the Usable Condition of Metallic Dies and Tools, of which the following is a full, clear, and complete

specification.

This invention relates to dies and tools made of steel and various steel alloys, and used for drop forgings, drawing, stamping, heading and otherwise shaping products of metal. These dies and tools are subjected to destructive wear by the shock, pressure, strain, etc., in the operation of the machines, in which they are used, and though made, as a rule, of the best quality of steel and steel alloys, the period of their usable condition is comparatively short. The object of my invention is to extend the period of their usable condition.

The efforts of producers of tool steels have been directed for many years to increase its toughness and otherwise improve its capacity to resist for a longer period the destructive effects, to which the dies for drop forgings, and tools for heading, drawing, etc., are exposed. My own researches and experiments were directed toward finding by what means, if any, the dies and tools made of the various steels, and steel alloys, may be maintained in usable condition for a longer period than heretofore. This led me to the discovery, that dies, punches and other similar tools for drop forging, heading and otherwise shaping of metallic parts, will, and do, withstand the destructive wear better, and for a much greater length of time, if they are artificially heated to, and kept heated while they are being used, at a temperature above their natural temperature and lower than that applied thereto in the hardening process. Roughly speaking this temperature at which the dies or tools are to be kept during their periods of active use varies from about 300 to about 1100° F., the degree of the temperature at which a die or tool is to be kept depending on the characteristics of the steel, or alloy, of which the die, tool, etc., is made. The tools or dies, made of some particularly compounded steels, and steel alloys, may have to be heated to, and kept at, a yet higher

temperature than the maximum stated above, but the rule, that the temperature is to be somewhat lower than that to which the material (steel or alloy) of which the die, or tool is produced, must be heated in 60 the hardening process, applies equally also to tools, or dies produced of these particularly compounded steels, or alloys.

To determine the temperature, which should, or may be, applied to a particular die or tool to attain the object of this invention, requires the knowledge of the composition of the steel, or alloy, of which the die, or tool is made, or of the temperature to which it must be heated in hardening it. 70 This information is readily obtainable from the maker of the steel or alloy, if not stated in the specifications, according to which the steel or alloy was produced. The examples here given are of steels and alloys 75 generally known and now used for the enumerated and similar work.

Considering first the ordinary straight carbon tool steels, largely used for drop forging dies, i. e. steels, containing from 0.75 80 to 0.90% carbon, and which are heated to 1400-1475° F. for hardening and whose tempering heat does not exceed 750° F., a very high degree of toughness and resistant 85 capacity is imparted to a die, or tool, produced of such a straight carbon steel, by heating it to, and keeping it while it is being used, at a temperature from about 400° to 600° F., the further rule being, in this instance, that the lighter the dropping 90 weight of the machine, in which the die or tool is being used, or the lighter the stock and the easier the metal flows, of which the drop forging is to be produced, the nearer to the stated lower limit of the temperature 95 the die may be heated and kept. I found also that it is preferable to heat and keep the tools or dies, made of straight carbon steels, at a lower temperature than tools or dies made of alloy steels, because the continuous application to the straight carbon tool steels of a temperature nearer to that to which they are heated in the hardening process will result in reducing their hardness.

105 Dies, or tools, made of steels alloyed with chrome nickel, carbon chromium, chrome vanadium, cobalt chromium, tungsten or molybdenum, will in some cases scarcely be affected by temperatures ranging up to 110

1100° F. This applies, for instance, to a tungsten high speed steel of approximately the following composition: C, 0.65; W, 16.00; Cr, 3.40; V, 0.80%. Tools, or dies, 5 made of the so-called "tungsten high speed steel" of this or similar composition for heavy forging, trimming and blanking will stand a much longer service if heated to 1100° F., and kept at that temperature while 10 they are being used. The period of their usable condition may be more than doubled thereby. Tools, or dies, made of cheaper grades of high speed steels, without any tungsten, for instance, a patented cobalt- 15 chromium combination, containing about:— C, 1.50; Co, 3.25; Cr, 12.00; Mo, 0.75%, may be kept at a temperature of about 850° F. without losing the required degree of their 20 hardness.

20 Dies for hydraulic bulldozing and compression work, as well as hot trimming and blanking, made of alloy steels containing approximately C, 0.45; W, 2.00; Cr, 1.00; Si, 0.80% if heated to about 500° F. and dies 25 and tools for hot trimming, drop forging and hot or cold bolt heading, produced of steel containing about C, 0.90; Mn, 0.40; Cr, 3.50; Si, 0.20%, will likewise their 30 usable condition maintained for a much longer period if heated to about 750° F. and kept at that temperature while they are being used.

The heating of these tools and dies and maintaining them so heated while being used, may be effected in various ways. One method that I have found to serve well for all temperatures, and may be said to be perhaps the simplest and most inexpensive means, is to apply, to the die, or tool, a jacket 35 tightly packed with infusorial earth in a layer of suitably thickness, and then heating it by gas burners. In this way the die or tool will be heated uniformly, and then kept heated at, or very near, the requisite temperature, for many hours. Fine molding sand may be used instead of the infusorial earth. Or, any approved form of electrical heating apparatus may be employed.

Where it is more convenient, and the die 40 or tool does not require to be heated above 600° F., an oil bath may take the place of

the packing of infusorial earth; or a bath of molten lead or a combination of lead and tin may be used. In this connection it is well to note that a compound of 14 parts of lead with 8 parts of tin melts at about 420° F., and a combination of 38 parts of lead with 8 parts of tin at about 510° F., these temperatures being required more frequently, and the molten condition of these 55 compounds serving to indicate the temperature of the die or tool.

The heating of the tool or die and the heat of the packing, or bath, are controlled by a suitable heat measuring instrument set 60 in a recess in the die or tool, in the packing, or in the bath, and provision may be made for continuously indicating the temperature of the dies or tools by providing suitable 65 temperature indicating instruments there- 70 for.

I claim as my invention:

1. The method of extending the period of usable condition of a metallic die or tool, which consists in artificially heating the die 75 or tool above the temperature naturally resulting from the use of the die or tool and below the temperature to which it was subjected in the hardening process, and keeping the die or tool at such temperature while it 80 is being used.

2. The method of extending the period of usable condition of a metallic die or tool, which consists in artificially heating the die 85 or tool to a temperature which will not impair its hardness but above the temperature naturally resulting from the use of the die or tool, and keeping the die or tool at such temperature while it is being used.

3. The combination with a metallic die, or 90 tool, of means for heating it, and for keeping it so heated while the die, or tool, is being used.

4. The combination with a metallic die, or tool, of means for heating it and of a pack- 95 ing for keeping it heated while the die or tool is being used.

HELLMUTH REINHARDT ROSENBAUM,

Witnesses:

CHARLES S. SKINNER,  
CHARLOTTE J. WATTON.